

## UNITED STATES PATENT OFFICE

2,371,221

## DYEING PROCESS

Robert Burns, Jackson Heights, N. Y., assignor to  
Celanese Corporation of America, a corporation  
of Delaware

No Drawing. Application September 26, 1942,  
Serial No. 459,825

13 Claims. (Cl. 8—61)

This invention relates to the treatment of materials and relates more particularly to the treatment of dyed materials such as fibers, threads, filaments or fabrics made of or containing organic derivatives of cellulose to obtain thereon colorations which are fast to acid fading.

An object of my invention is to treat colored fabrics of organic derivative of cellulose textile materials which have been dyed with colors ordinarily not fast to acid fumes to inhibit the fading of said dyed materials when exposed to such fumes.

Other objects of my invention will appear from the following detailed description.

In the coloration of textile materials it is very desirable that the colors produced on the materials be as fast as possible to light, washing and to other agencies such as acid fumes. Many dyestuffs yield on organic derivative of cellulose materials desirable shades which are fast to washing but these dyestuffs often suffer from a lack of fastness to acid fumes. When fabrics to which these dyestuffs have been applied are exposed to acid fumes, for example, the products of combustion of coal, gas, etc., the color undergoes a change in shade. This change is usually referred to as acid fading. The change which occurs may be a dulling of the brightness of the shade in some instances, and in others there may be a definite change in color. This undesirable effect is frequently observed in the case of many anthraquinone dyestuffs which yield valuable blue colors on organic derivative of cellulose materials. When fabrics dyed with these colors are exposed to acid fumes the colors change from a pure blue shade to one having a reddish cast. On continued exposure to the acid fumes the blue color may even change to a pink color. Such changes naturally restrict the range of usefulness of these dyestuffs and methods of increasing the resistance of these dyes to acid fading are of great commercial importance.

I have now discovered that the acid fading characteristics of organic derivative of cellulose textile materials dyed with water-insoluble anthraquinone dyestuffs of the dispersol type may be substantially improved. These desirable results may be achieved if such dyed textile materials are treated with tannic acid so that the tannic acid is precipitated and retained within the structure of the material in the form of an insoluble tannate. When dyed textile materials are treated in this way, the dyed material obtained exhibits excellent resistance to acid fading and

the textile material may be exposed to acid fumes for substantial periods with little or no effect upon the color of the material.

The insoluble tannate may be precipitated within the dyed textile materials in several ways. This may be done, for example, by first impregnating the material with a solution of tannic acid, then treating the impregnated material with a solution or suspension of a metal compound which reacts with the tannic acid to form an insoluble tannate. Conversely, the dyed textile material may first be treated with a solution or suspension of a metal compound which is capable of reacting with tannic acid to form an insoluble tannate, and the treated textile material may then be padded or otherwise impregnated with a solution of tannic acid to form the insoluble tannate. Compounds of metals such as, for example, calcium, magnesium, iron and manganese all may be employed to form water-insoluble tannates.

In treating the dyed organic derivative of cellulose textile materials, it is preferable that the textile material be dried after being impregnated with either the tannic acid or the metal compound prior to the formation and precipitation of the tannate. Thus, when treating fabrics the latter may be padded with a solution or suspension of the metal compound or of tannic acid, which may be maintained at a temperature of from 20 to 100° C. After being padded, the fabric may be dried by passing through a drying chamber through which air heated to 85 to about 120° C. is circulated. After the fabric is dried, the insoluble tannate is formed in the treated textile material by padding it with a solution of tannic acid if the initial treatment was with a metal compound, or by padding with a solution or suspension of a metal compound if the initial padding was with a solution of tannic acid.

The solutions employed for treating the dyed organic derivative of cellulose textile materials may be of varying concentrations. In the case of tannic acid the solution may be of a concentration of from 0.1 to 10% by weight, optimum results, however, being achieved with solutions of concentrations of about 0.5% by weight. The solutions or suspensions of the metal compound which are employed may contain from about 0.5 to 20% or more by weight of the metal compound depending upon the concentration of the tannic acid solution with which it is to be reacted. Thus, for example, when calcium hydroxide is employed as the metal compound to form insoluble

ble calcium tannate, an aqueous suspension comprising about 1% by weight of the metal compound yields the desired result.

Wetting, dispersing and softening agents may also be added to the tannic acid solutions as well as to the solutions or suspensions of the metal compounds to improve penetration and to yield a more uniformly treated product. Such wetting or dispersing agents may be sulfonated oils, sulfated long chain fatty alcohols, sulfonated fatty acid esters, alkyl substituted aryl sulfonates, and the like.

The amount of insoluble tannate precipitated in the dyed organic derivative of cellulose textile material in accordance with my invention may be from about 0.1 to 10% on the weight of the fabric or other textile material.

In order further to illustrate my invention but without being limited thereto, the following examples are given.

*Example I*

A cellulose acetate fabric dyed in a blue shade with 1% of 1:4 di-methylamino-anthraquinone is padded with a 0.5% solution of tannic acid at 40° C. and dried. The dried fabric is then padded with a suspension containing 1% by weight of calcium hydroxide. The reaction between the calcium hydroxide and the tannic acid causes an insoluble precipitate of calcium tannate to form in the fabric. The fabric is washed for 10 minutes at 70° C. and then exposed to an atmosphere containing acid fumes. After 40 hours exposure the color of the treated fabric is altered only slightly, the change being only that the color now has a slight reddish cast. Untreated dyed fabric exposed for 40 hours to the same acid conditions undergoes a complete change of color, the blue fading to a pink color.

*Example II*

A cellulose acetate fabric dyed as in Example I is padded with a 1% solution of calcium hydroxide at 40° C. and dried. The dried fabric is then padded with a 0.5% solution of tannic acid which reacts with the calcium hydroxide to form insoluble calcium tannate in the fabric. After treatment the fabric is washed for 10 minutes at 70° C. The treated fabric is then exposed to an acid atmosphere for 40 hours with only a slight change in shade, i. e. a slight reddish cast on the blue color, while untreated dyed fabric changes completely from the original blue shade to a pink under like conditions of exposure.

*Example III*

A cellulose acetate fabric dyed as in Example I is padded with a 1% solution of calcium hydroxide at 40° C. and dried. The dried fabric is then padded with a 0.5% solution of tannic acid containing 2% by weight of "Parapon R," an agent comprising a highly sulfonated fatty acid ester and a softener, which softener is likewise a sulfonated fatty acid ester. After treatment, the fabric is washed. The treated dyed fabric is strongly resistant to acid fading and shows little change after a 40 hour exposure to acid fumes.

While my invention has been more particularly described in connection with the treatment of cellulose acetate textile materials, other organic derivative of cellulose textile materials, such as cellulose esters and cellulose ethers, may likewise be treated in accordance with the process of my invention. Examples of cellulose esters are cellulose propionate and cellulose butyrate, and

mixed esters such as cellulose acetate-propionate and cellulose acetate-butyrate, while examples of cellulose ethers are ethyl cellulose and benzyl cellulose. Not only may dyed fabrics be treated to improve their resistance to acid fading, but the acid fading characteristics of dyed textile materials in other forms, such as, for example, yarns and filaments in the form of hanks or wound on bobbins, or staple fiber in the form of a top may likewise be improved by my novel treatment.

The term "water-insoluble anthraquinone dyes of the dispersol type" as herein used applies to any water-insoluble dye of the anthraquinone series that can be employed in the dispersed state for coloring cellulose acetate or other organic derivative of cellulose textile material.

It is to be understood that the foregoing detailed description is merely given by way of illustration and that many variations may be made therein without departing from the spirit of my invention.

Having described my invention, what I desire to secure by Letters Patent is:

1. Process for improving the fastness to acid fumes of colorations on organic derivative of cellulose textile materials dyed with water-insoluble anthraquinone dyes of the dispersol type, which comprises forming a water-insoluble tannic acid salt of a metal on said colored organic derivative of cellulose textile material.

2. Process for improving the fastness to acid fumes of colorations on cellulose acetate textile materials dyed with water-insoluble anthraquinone dyes of the dispersol type, which comprises forming a water-insoluble tannic acid salt of a metal on said colored cellulose acetate textile material.

3. Process for improving the fastness to acid fumes of colorations on cellulose acetate textile materials dyed with water-insoluble anthraquinone dyes of the dispersol type which comprises forming calcium tannate on said colored cellulose acetate textile material.

4. Process for improving the fastness of colorations on organic derivative of cellulose textile materials dyed with water-insoluble anthraquinone dyes of the dispersol type to acid fumes, which comprises impregnating said dyed textile material with a solution of tannic acid, drying the impregnated material, and treating said dried material with a solution of a metal compound adapted to react with said tannic acid and form a water-insoluble metal tannate thereon.

5. Process for improving the fastness of colorations on organic derivative of cellulose textile materials dyed with water-insoluble anthraquinone dyes of the dispersol type to acid fumes, which comprises impregnating said dyed textile material with a solution of a metal compound which forms a water-insoluble tannic acid salt on reaction with tannic acid, drying the impregnated material, and treating the dried material with a solution of tannic acid.

6. Process for improving the fastness of colorations on cellulose acetate textile materials dyed with water-insoluble anthraquinone dyes of the dispersol type to acid fumes, which comprises impregnating said dyed textile material with a solution of tannic acid, drying the impregnated material, and treating said dried material with a solution of a metal compound adapted to react with said tannic acid and form a water-insoluble metal tannate thereon.

7. Process for improving the fastness of colora-

tions on cellulose acetate textile materials dyed with water-insoluble anthraquinone dyes of the dispersol type to acid fumes, which comprises impregnating said dyed textile material with a solution of a metal compound which forms a water-insoluble tannic acid salt on reaction with tannic acid, drying the impregnated material and treating the dried material with a solution of tannic acid.

8. Process for improving the fastness of colorations on a cellulose acetate fabric dyed with water-insoluble anthraquinone dyes of the dispersol type to acid fumes, which comprises padding said fabric with a solution of tannic acid, drying the treated fabric, and padding said dried fabric with a suspension of calcium hydroxide to form a water-insoluble calcium tannate on said dyed fabric.

9. Process for improving the fastness of colorations on a cellulose acetate fabric dyed with water-insoluble anthraquinone dyes of the dispersol type to acid fumes, which comprises padding said dyed fabric with a suspension of calcium hydroxide, drying the treated fabric, and padding said dried fabric with a solution of tannic acid to form a water-insoluble tannate on said dyed fabric.

10. Process for improving the fastness of col- 25

orations on a cellulose acetate fabric dyed with water-insoluble anthraquinone dyes of the dispersol type to acid fumes, which comprises padding said dyed fabric with a suspension of calcium hydroxide, drying the treated fabric, and padding said dried fabric with a solution of tannic acid containing a wetting and softening agent to form a water-insoluble calcium tannate on said dyed fabric.

11. Organic derivative of cellulose textile materials dyed with water-insoluble anthraquinone dyes of the dispersol type having improved fastness to acid fumes and having incorporated therein a water-insoluble tannate of a metal.

12. Cellulose acetate textile materials dyed with water-insoluble anthraquinone dyes of the dispersol type having improved fastness to acid fumes and having incorporated therein a water-insoluble tannate of a metal.

13. Cellulose acetate textile material dyed with a water-insoluble anthraquinone dyestuff of the dispersol type having improved fastness to acid fumes and having calcium tannate incorporated therein.

ROBERT BURNS.

CERTIFICATE OF CORRECTION.

Patent No. 2,371,221.

March 13, 1945.

ROBERT BURNS

It is hereby certified that error appears in the printed specification of the above numbered patent requiring correction as follows: Page 3, first column, line 25, claim 9, before the word "tannate" insert --calcium--; and that the said Letters Patent should be read with this correction therein that the same may conform to the record of the case in the Patent Office.

Signed and sealed this 5th day of June, A. D. 1945.

Leslie Frazer

Acting Commissioner of Patents.

(Seal)

tions on cellulose acetate textile materials dyed with water-insoluble anthraquinone dyes of the dispersol type to acid fumes, which comprises impregnating said dyed textile material with a solution of a metal compound which forms a water-insoluble tannic acid salt on reaction with tannic acid, drying the impregnated material and treating the dried material with a solution of tannic acid.

8. Process for improving the fastness of colorations on a cellulose acetate fabric dyed with water-insoluble anthraquinone dyes of the dispersol type to acid fumes, which comprises padding said fabric with a solution of tannic acid, drying the treated fabric, and padding said dried fabric with a suspension of calcium hydroxide to form a water-insoluble calcium tannate on said dyed fabric.

9. Process for improving the fastness of colorations on a cellulose acetate fabric dyed with water-insoluble anthraquinone dyes of the dispersol type to acid fumes, which comprises padding said dyed fabric with a suspension of calcium hydroxide, drying the treated fabric, and padding said dried fabric with a solution of tannic acid to form a water-insoluble tannate on said dyed fabric.

10. Process for improving the fastness of col- 25

orations on a cellulose acetate fabric dyed with water-insoluble anthraquinone dyes of the dispersol type to acid fumes, which comprises padding said dyed fabric with a suspension of calcium hydroxide, drying the treated fabric, and padding said dried fabric with a solution of tannic acid containing a wetting and softening agent to form a water-insoluble calcium tannate on said dyed fabric.

11. Organic derivative of cellulose textile materials dyed with water-insoluble anthraquinone dyes of the dispersol type having improved fastness to acid fumes and having incorporated therein a water-insoluble tannate of a metal.

12. Cellulose acetate textile materials dyed with water-insoluble anthraquinone dyes of the dispersol type having improved fastness to acid fumes and having incorporated therein a water-insoluble tannate of a metal.

13. Cellulose acetate textile material dyed with a water-insoluble anthraquinone dyestuff of the dispersol type having improved fastness to acid fumes and having calcium tannate incorporated therein.

ROBERT BURNS.

CERTIFICATE OF CORRECTION.

Patent No. 2,371,221.

March 13, 1945.

ROBERT BURNS

It is hereby certified that error appears in the printed specification of the above numbered patent requiring correction as follows: Page 3, first column, line 25, claim 9, before the word "tannate" insert --calcium--; and that the said Letters Patent should be read with this correction therein that the same may conform to the record of the case in the Patent Office.

Signed and sealed this 5th day of June, A. D. 1945.

Leslie Frazer

Acting Commissioner of Patents.

(Seal)